



US006755722B1

(12) **United States Patent**  
Horie et al.

(10) **Patent No.:** **US 6,755,722 B1**  
(45) **Date of Patent:** **Jun. 29, 2004**

(54) **METHOD OF CHEMICAL MECHANICAL TEXTURING**

(75) Inventors: **Yuji Horie**, Tokyo (JP); **Takabumi Marukawa**, Tokyo (JP); **Kanichi Endo**, Tokyo (JP)

(73) Assignee: **Nihon Microcoating Co., Ltd.**, Tokyo (JP)

(\*) Notice: Subject to any disclaimer, the term of this patent is extended or adjusted under 35 U.S.C. 154(b) by 0 days.

(21) Appl. No.: **09/590,643**

(22) Filed: **Jun. 8, 2000**

(30) **Foreign Application Priority Data**

Jun. 24, 1999 (JP) ..... 11-178258  
(51) **Int. Cl.** <sup>7</sup> ..... **B24B 1/00**  
(52) **U.S. Cl.** ..... **451/41; 451/59; 451/63**  
(58) **Field of Search** ..... **451/41, 36, 59, 451/63, 307**

(56) **References Cited**

U.S. PATENT DOCUMENTS

4,973,496 A \* 11/1990 Kruger et al. ..... 427/129

5,482,497 A \* 1/1996 Gonnella et al. ..... 451/57  
5,593,341 A \* 1/1997 Gonnella et al. ..... 451/57  
5,879,222 A \* 3/1999 Robinson ..... 451/41  
5,899,794 A \* 5/1999 Shige et al. ..... 451/41  
5,906,804 A \* 5/1999 Aral et al. ..... 423/265  
6,099,604 A \* 8/2000 Sandhu et al. ..... 51/307  
6,258,721 B1 \* 7/2001 Li et al. ..... 438/693  
6,315,638 B1 \* 11/2001 Marukawa ..... 451/36  
6,491,572 B1 \* 12/2002 Horie et al. ..... 451/63

\* cited by examiner

*Primary Examiner*—M. Rachuba

(74) *Attorney, Agent, or Firm*—Beyer Weaver & Thomas LLP

(57) **ABSTRACT**

Minute and uniform line marks can be formed on the surface of a glass substrate for a magnetic disk by pressing a woven cloth tape comprising plastic fibers preferably by a rubber roller with hardness greater than 60 and causing it to run thereover while supplying a suspension containing abrading particles and a solution which contains hydroxyl groups such as a KOH solution.

**4 Claims, 1 Drawing Sheet**





Fig.1

## METHOD OF CHEMICAL MECHANICAL TEXTURING

### BACKGROUND OF THE INVENTION

This invention relates to a method of texturing the surface of a glass substrate for a magnetic disk and more particularly to a method of chemical mechanical texturing for a surface of such a glass substrate.

The substrate of a magnetic disk has its surface mirror polished first and then has it textured so as to have a specified surface roughness. The purpose of texturing is to form line marks on the substrate surface such that when it is used with a magnetic head, the floating distance of the magnetic head from the disk surface can be maintained dependably constant while the disk is rotating at a fast rate and also such that the magnetic head can be prevented from becoming adsorbed to the disk surface while the disk is stationary.

The texturing is usually carried out by supplying a suspension mixed with minute abrasive particles of diamond or alumina to the surface of the substrate while the latter is rubbed with- a woven or unwoven tape or a tape with planted piles. Textured line marks can thus be formed as these abrading particles are pressed on and rubbed against the substrate surface to mechanically grind it. Such a process for forming line marks is usually referred to as the chemical mechanical texturing.

Recently, glass substrates are coming to be used as commonly as substrates made of an aluminum alloy for producing magnetic disks, and these glass substrates are also required to have their surface or surfaces textured for the same reasons, that is, such that the floating distance of the magnetic head can be reduced and hence that the recording density of the magnetic disks as memory media can be increased.

Since glass substrates are hard, however, it has been considered difficult to form sufficiently minute and uniform line marks on a glass substrate by a mechanical texturing process,

### SUMMARY OF THE INVENTION

It is therefore an object of this invention to provide a chemical mechanical texturing method by which minute and uniform line marks can be formed on the surface of a glass substrate for a magnetic disk.

The chemical mechanical texturing method embodying this invention, with which the above and other objects can be accomplished, may be characterized by the steps of pressing a woven cloth tape made of plastic fibers against a surface of a glass substrate and causing it to run thereover while supplying thereonto a suspension containing abrading particles and a solution which contains hydroxyl groups.

If a method according to this invention is used, the solution in the suspension containing hydroxyl groups causes a solid phase reaction on the contact boundary surface between the abrading particles in the suspension and the surface of the glass substrate, thereby generating over this surface a substance which is different and the texturing process is carried out while this boundary surface portion is chemically and mechanically removed. Since the method makes use of this chemical reaction on the surface of the glass substrate caused by the solution containing hydroxyl groups in the suspension, deterioration or degradation due to the process is negligible and since work units of the process are extremely small, it is possible to form extremely small line marks.

The solution in the suspension containing hydroxyl groups serves not only to accelerate the chemical polishing process due to the solid-phase reaction which takes place over the contact surfaces between the abrading particles and the substrate surface but also as a coolant, absorbing the heat of friction due to the mechanical grinding process between the abrading particles and the glass substrate.

Examples of solution containing hydroxyl groups suitable for the purpose of this invention includes KOH and NaOH 10 solutions.

### BRIEF DESCRIPTION OF THE DRAWINGS

FIG. 1, which is incorporated in and forms a part of this specification, schematically illustrates a texturing machine 15 which may be used in a method embodying this invention.

### DETAILED DESCRIPTION OF THE INVENTION

FIG. 1 shows a texturing machine which may be suitably used for the purpose of this invention.

A liquid suspension L containing abrading particles and hydroxyl groups is supplied through a nozzle N onto the surface of a glass substrate D while the glass substrate D is 25 rotated in the direction indicated by arrow R and a woven cloth tape T made of plastic fibers is caused to travel in a reverse direction indicated by arrow M (opposite the direction R) to carry out a chemical mechanical texturing process. Such a woven cloth tape T may be prepared by slicing into the shape of the tape a woven or knit cloth of plastic fibers with high tensile strength and resistance against chemicals such as polyester, nylon or polyethylene fibers. The thickness of the woven cloth tape T is within the range of 5  $\mu\text{m}$ -5000  $\mu\text{m}$ .

The glass substrate D is rinsed immediately after the woven cloth tape T is retracted from the glass substrate D by 35 flowing a rinsing liquid on the surface of the glass substrate D without removing it from the texturing machine.

If a texturing machine as shown in FIG. 1 is used, the woven cloth tape T is pressed against the glass substrate D by means of a rubber roller P. The durometer hardness of the rubber roller should be at least 60 degrees since line marks would not be formed on the surface of the glass substrate D if the hardness of the rubber roller P were too low.

The liquid suspension to be used for the purpose of this invention may be obtained by adding a solution containing hydroxyl groups such as KOH and NaOH solutions into an aqueous solution in which abrading particles are dispersed, 50 Examples of abrading particles suitable for the purpose of this invention include particles of diamond, silicon carbide, alumina and zirconia with diameters in the range of 0.01  $\mu\text{m}$ -5  $\mu\text{m}$  which are commonly used for grinding and polishing.

The invention is described next by way of the results of test and comparison experiments carried out by the inventors in which glass substrates for magnetic disks were textured and the surface roughness after the processing was measured.

For the test experiment, use was made of a woven cloth tape of thickness 75  $\mu\text{m}$ , prepared by slicing a woven cloth comprising polyester fibers of thickness 1.0 denier into the shape of a tape. The suspension was prepared by adding 5 weight % of KOH to 95 weight % of aqueous solution 60 containing diamond particles of diameter 2  $\mu\text{m}$  (with 0.5 weight % of diamond particles and 99.5 weight % of pure water).

**3**

A polishing machine as shown in FIG. 1 was used under the following conditions:

Speed of rotation of the glass substrate=100 rpm;

Speed of travel of the tape=10 cm/min;

Hardness (durometer hardness) of the rubber roller=80 degrees;

Force of pressure=2.27 kg;

Suspension supply rate=10 ml/min; and

Time of polisher operation=30 seconds.

The surface roughness Ra of the glass substrate used for the texturing experiment was 3.0 Å before the polishing.

After the chemical mechanical texturing as described above, a scanning probe microscope (Nanoscope Dimension 3100 Series produced by Digital Instrument, Inc.) was used to scan (at 256 points) a randomly selected area of 30  $\mu\text{m} \times 30 \mu\text{m}$  on the surface of the glass substrate. The measured average surface roughness over this selected area was 4.4 Å.

The surface condition of the glass substrate was observed and it was ascertained that textured line marks were uniformly formed thereon.

A comparison experiment was carried out on a similar glass substrate with a mirror-polished surface of which the initial average surface roughness was also 3.0 Å by using another rubber roller with hardness 40. As in the test experiment described above, the average surface roughness of the glass substrate was measured after the texturing over a randomly selected surface area of 30  $\mu\text{m} \times 30 \mu\text{m}$ . The measured surface roughness after the texturing was 3.6 Å.

**4**

Line marks were not formed uniformly on the polished substrate surface. What was accomplished was that the substrate surface was polished to an approximately uniform surface roughness.

The results of these experiments clearly show that uniform line marks can be formed on the surface of a glass substrate by a method according to this invention.

What is claimed is:

1. A method of chemical mechanical texturing comprising the steps of:

supplying a suspension comprising abrading particles and a solution containing hydroxyl groups onto a surface of a glass substrate; and

texturing said surface by simultaneously pressing a woven cloth tape comprising plastic fibers and free of planted piles onto said surface and carrying out a chemical mechanical texturing on said glass substrate by causing said tape to travel over said surface, wherein said woven cloth tape is pressed against said surface with a rubber roller with durometer hardness greater than 60 degrees.

2. The method of claim 1 wherein said solution comprises KOH.

3. The method of claim 1 wherein said abrading particles have diameters 0.01  $\mu\text{m}$ -5  $\mu\text{m}$ .

4. The method of claim 1 wherein said plastic fibers are polyester fibers.

\* \* \* \* \*